

D. M. BARRINGER.

SEPARATION OF MAGNETIC IRON ORE FROM ITS ASSOCIATED NON-MAGNETIC OR FEEBLY  
MAGNETIC MINERALS.

APPLICATION FILED MAY 10, 1911. RENEWED JULY 17, 1917.

1,256,972.

Patented Feb. 19, 1918.

2 SHEETS—SHEET 1.

FIG. I.



FIG. II.



Inventor

Daniel Moreau Barringer,

*Stalley & Pang*

Attorneys.

Witnesses  
John C. Berger  
James H. Bell

D. M. BARRINGER.

SEPARATION OF MAGNETIC IRON ORE FROM ITS ASSOCIATED NON-MAGNETIC OR FEEBLY  
MAGNETIC MINERALS.

APPLICATION FILED MAY 10, 1911. RENEWED JULY 17, 1917.

1,256,972.

Patented Feb. 19, 1918.

2 SHEETS—SHEET 2.



Inventor

Daniel Moreau Barringer

by *J. G. Bergner*  
*Julley + Lang*

Attorney

Witnessed  
*John G. Bergner*  
*James D. Bell*

# UNITED STATES PATENT OFFICE.

DANIEL M. BARRINGER, OF WAYNE, PENNSYLVANIA.

## SEPARATION OF MAGNETIC IRON ORE FROM ITS ASSOCIATED NON-MAGNETIC OR FEEBLY-MAGNETIC MINERALS.

1,256,972.

Specification of Letters Patent. Patented Feb. 19, 1918.

Application filed May 10, 1911, Serial No. 626,291. Renewed July 17, 1917. Serial No. 181,176.

To all whom it may concern:

Be it known that I, DANIEL M. BARRINGER, of Wayne, in the county of Delaware and State of Pennsylvania, have invented certain new and useful Improvements in the Separation of Magnetic Iron Ore from Its Associated Non-Magnetic or Feebly-Magnetic Minerals, whereof the following is a specification, reference being had to the accompanying drawings.

My invention relates to a process of separation which is carried out by suspending the mixed materials in finely divided state over the pole of an electro-magnet energized by an alternating current, with interposition of a plate of electrically conductive material. When this is done, especially if the material be agitated to assist the separation, the magnetic material, as for example, magnetic iron ore, travels constantly toward the edge of the plate, with an appearance as though repelled from the pole of the electro-magnet beneath the separating plate. My process for the utilization of this behavior of magnetic material in order to effect its separation is to cause the mixed material in a properly divided state to travel constantly, preferably with concomitant agitation, down an inclined trough of electrically conductive material, (or with such material immediately below it), beneath which is placed a series of electro-magnets energized by an alternating electric current. Under these circumstances, the magnetic materials are caused to continuously travel to and as it were climb over the dividing ridges which form the edges of the trough.

In order to illustrate the process which I have invented, I have shown and will briefly describe an apparatus conveniently devised for the practice of the process.

In the accompanying drawings, Figure I, is a plan view of such an apparatus for the practice of the process.

Fig. II, is a longitudinal view thereof.

Fig. III, is a cross sectional view thereof.

The apparatus shown in Fig. I, comprises a series of disconnected inclined central troughs 1, 1, of copper or other electrically conductive material, preferably of considerable thickness. At the end of each trough is a discharge space 10. Underneath these troughs and in the plane of the median line thereof, are a series of electro-magnets 2, 2, 2, energized by an alternating electric current derived from a generator indicated at

G in Fig. II of the drawings. This generator is connected through a suitable line 1 to the magnets 2, 2, 2.

Each trough 1, overlaps at both edges, 60 and thereby forms a practically continuous surface with the side trough 4, 4, with formation of dividing or intervening ridges 11, 11, between them. Beyond the lower end of the trough 1, the side troughs 4, 4, converge and discharge into the next succeeding central trough. Above the edges of the central troughs are suspended longitudinal pipes 5, 5, from which a series of water or air jets are directed toward the ridges 70 formed where the edges of the central trough overlap the side troughs, which jets serve to mechanically facilitate the travel into the side trough of the separated magnetic material which the magnetic action or 75 flux has caused to advance to the edge of the central trough.

In employing this apparatus in the practice of my process comminuted magnetic iron ore with its associated minerals is directed into the upper end of the uppermost central trough down which it is carried by a stream of water. As the mixed materials pass over the electro-magnets the particles of magnetic iron ore travel continuously and 85 constantly toward the edges of the trough, and climb against gravity over the dividing ridges into the said troughs, while the non-magnetic or feebly magnetic gangue passes on and is discharged through the discharge 90 space 10, at the lower extremity of each central trough. The magnetic ore which has climbed the ridges of the central trough, passes on assisted by the jets of water into the side troughs, where the water flowing 95 down these troughs carries the material into the central trough next below in the series, where the operation is repeated, resulting in successive separations, continued until a pure residuum is obtained, the degree of 100 purity depending upon the number of times that it is found desirable to repeat the operation. The water not only serves to convey the material down to the trough, but it also has a tendency to make the particles of the 105 mixture stand apart as they pass through the magnetized portion of the separator and the magnetic particles, therefor, more easily detach themselves from the gangue.

I find that the process of separation is 110 facilitated by the employment of a circuit breaker in connection with the current by

which the magnets are energized, so as to make and break the current at short intervals. For this purpose an interrupter, indicated at I in Fig. II of the drawings, may 5 be used. This appears to occasion additional agitation of the ore and prevents the accidental mechanical carrying over of non-magnetic particles by the magnetic particles as they climb over the dividing ridges into 10 the side troughs. It will be understood that the number of the separators in the entire series may be increased as circumstances dictate.

It also will be understood that the effectiveness of my apparatus depends upon the proper management of a large number of readily controllable factors. Thus, (a) the central metal trough may vary in thickness and may be made of copper, aluminum, or 15 other metal or alloy thereof. (b) The slopes of the sides of the trough, and its width may be varied. (c) The angle of inclination of the trough may be varied so as to regulate the rapidity of flow of material. This may be readily accomplished 20 by a suitable cam, indicated at C in Fig. II of the drawings. (d) The strength of the electro-magnets or their distance from the bottom of the trough may be varied. (e) 25 The strength or the frequency of the electric current may be varied. (f) The rate at which the material or the water may be fed to the apparatus may vary. (g) The frequency with which the current is interrupted by the circuit-breaker may vary.

All of these factors play their part in effecting the separation of the ore. They may all be readily varied. By such variation a very accurate regulation and control 40 of the process is secured. By carrying out the process by the use of a number of successive separators such as I have described, and by varying the above named factors as between successive separators, I am able 45 to secure a very delicate regulation of the process so that I may not merely separate magnetic from non-magnetic materials in the broader use of the terms, but I may after such separation further separate highly 50 magnetic from feebly magnetic materials, as for example, magnetite from ilmenite.

Although I have spoken of the magnetic iron ore as being repelled from the pole by reason of the interposition of the electrically 55 conductive plate, yet I wish it to be understood that I am merely speaking of appearances. I do not here undertake to give any explanation of the phenomena which occur.

Having thus described my invention, I 60 claim:—

1. The process of separating magnetic ma-

terials from non-magnetic materials, which consists in subjecting the magnetic materials traveling with the non-magnetic materials by gravity on a substantially non-magnetic 65 plate of high electrical conductivity to the influence of magnetic flux created by an electro-magnet energized by an alternating current of electricity, and thereby diverting the magnetic particles from their normal path 70 of travel through the influence of the magnetic flux thereon.

2. The process of separating magnetic materials from non-magnetic materials, which consists in subjecting the magnetic materials 75 traveling with the non-magnetic materials by gravity on a substantially non-magnetic plate of high electrical conductivity to the influence of magnetic flux created by an electro-magnet having a fixed position relative 80 to said plate and energized by an alternating current of electricity, and thereby diverting the magnetic particles from their normal path of travel through the influence 85 of the magnetic flux thereon.

3. The process of separating magnetic from non-magnetic materials which consists in conveying the mixed materials by water down an inclined trough of substantially non-magnetic material of high electrical 90 conductivity, and subjecting said materials to the influence of a magnetic flux created by an electro-magnet energized by an alternating current of electricity, the water acting to separate the particles and reduce the 95 friction of the same on the trough and on each other, whereby said magnetic materials are caused to be separated from the non-magnetic materials and travel toward the edges of the trough and over the same. 100

4. The process of separating magnetic materials from materials which are less magnetic, which consists in causing both materials to travel on a substantially non-magnetic plate of high electrical conductivity, 105 and simultaneously subjecting them to the influence of magnetic flux, created by an electro-magnet energized by an alternating current of electricity, said electro-magnet being situated upon the opposite side of 110 the conducting plate from the traveling materials, whereby the magnetic particles are diverted from their normal path of travel, through the influence of magnetic flux thereon.

In testimony whereof, I have hereunto signed my name at Philadelphia, Pennsylvania, this sixth day of May, 1911.

DANIEL M. BARRINGER.

Witnesses:

HENRY T. BECKWITH,  
JAMES H. BELL.